

# UNITED STATES PATENT OFFICE.

GEORGE STEELE DUNCAN AND GEORGE HENRY POTTS, OF EDINBURGH,  
SCOTLAND, ASSIGNORS TO AMERICAN OFFSET COMPANY, OF NEW  
YORK, N. Y., A CORPORATION OF NEW YORK.

## COMPOSITION FOR PREVENTING SET-OFFS IN PRINTING.

No. 823,676.

Specification of Letters Patent.

Patented June 19, 1906.

Application filed August 7, 1905. Serial No. 273,140.

*To all whom it may concern:*

Be it known that we, GEORGE STEELE DUNCAN and GEORGE HENRY POTTS, subjects of the King of the United Kingdom of Great Britain and Ireland, residing at Edinburgh, Scotland, have invented certain new and useful Improvements in Compositions for Preventing Set-Offs in Printing, of which the following is a specification.

10 In the specification of application Serial No. 259,374 is described a liquid composition to be used for damping the "set-off" rollers in printing-machines to prevent set-off or transfer of ink from one sheet to another or 15 from one side to the reverse side of a sheet in printing.

Our present invention has for its object the provision of a liquid composition to be used in the same manner as the liquid composition 20 the subject of the said application, but differing therefrom in its composition and possessing especial advantages if some or all of the work is to be done on high-speed rotary machines.

25 The constituents of the liquid composition the subject of our present invention are palm-oil or whale-oil, or both, lard-oil or cocoanut-oil, or both, with or without all or any of the following oils: sperm-oil, tallow-oil, cotton-seed oil, and soap, preferably brown windsor soap, spirits of wine, naphtha, and turpentine, the two last as ordinarily used by printers. Whale-oil is the equivalent of palm-oil for use in our composition. Similarly, cocoanut-oil is the equivalent of lard-oil. Where one is mentioned, the equivalent may be used or a mixture of the equivalent oils. In like manner sperm, tallow, and cotton-seed oil are equivalent, and either or all may be 40 used with like result in our composition.

The best proportions are the following: The volume of the palm-oil or whale-oil or of the mixture of both should be about the same as the volume of the lard-oil or cocoanut-oil 45 or of the mixture of both, and the volume of each of the oils—sperm, tallow, and cotton-seed oils—if used should not exceed the half of the volume of the palm or whale oils or of the mixture of these two oils. The soap

should be about one pound to about three pints of palm or whale oil or of the mixture of these two. The spirits of wine and turpentine should be about in equal volumes, and the volume of each should be rather more than half, say, two-thirds, the volume of the palm or whale oils or of the mixture of these two. The naphtha should be twice as much, by volume, as the turpentine and may be even appreciably more than twice such volume. It is preferable to use some sperm-oil to assist admixture. If cotton-seed oil is dispensed with or its volume diminished, the volume of the lard-oil or cocoanut-oil or of the mixture of these two should be proportionately increased. The volumes of such of the above-mentioned oils as are solid at ordinary temperatures are measured after by gentle heating the particular oils have been liquefied.

As it is desirable to apply heat to effect as good an admixture of the soap as possible and accordingly to defer adding the naphtha until after such heating, we have found it preferable, especially if the heating is done, for example, over an open fire, to employ the method described in the specification of the said application in effecting the mixture of the components of the liquid composition the subject of our present invention. Instead of naphtha benzin may be used, but naphtha is preferable.

Having now described our invention, what we claim, and desire to secure by Letters Patent of the United States, is—

1. A composition for preventing set-off comprising palm-oil, lard-oil, soap, spirits of wine, naphtha, and turpentine.

2. A composition for preventing set-off comprising palm-oil, lard-oil, sperm-oil, soap, spirits of wine, naphtha and turpentine.

In testimony whereof we have signed our names to this specification in the presence of two subscribing witnesses.

GEORGE STEELE DUNCAN.  
GEORGE HENRY POTTS.

Witnesses:

MARY McCREDIE,  
WALLACE CRANSTON FAIRWEATHER.